

# UNITED STATES PATENT OFFICE.

JOHANNES KORSELT, OF ZITTAU, GERMANY, ASSIGNOR, BY MESNE ASSIGNMENTS, TO  
THE CHEMICAL FOUNDATION, INC., A CORPORATION OF DELAWARE.

## METHOD OF RENDERING ANIMAL AND VEGETABLE FIBERS ACTIVE.

1,426,298.

Specification of Letters Patent. Patented Aug. 15, 1922.

No Drawing.

Application filed October 24, 1917. Serial No. 198,337.

*To all whom it may concern:*

Be it known that I, JOHANNES KORSELT, a citizen of the German Empire, residing at Zittau, Saxony, Germany, have invented 5 certain new and useful Improvements in a Method of Rendering Animal and Vegetable Fibers Active (for which I have filed an application in Germany August 19, 1916), of which the following is a specification.

10 My invention relates to a method of treating animal and vegetable fibers such as wool, hairs, feathers and cotton with a view to rendering them active either in a coloured or uncoloured condition.

15 With this object in view my invention consists in treating the fibers with suitable ferments which are devoid of any colouring matter.

I have ascertained that certain ferments 20 such as catalase confer upon silk certain valuable properties and that by treating other fibers either animal or vegetable, such as wool, hairs, feathers, cotton, artificial silk and the like, with such ferments one 25 succeeds in rendering these fibers active. If wool for instance is treated with catalase, its strength and elasticity, as well as its power of absorbing colouring matter, is greatly increased. Wool which contains 30 so-called dead hairs not well adapted to be coloured, is rendered active upon being treated with suitable ferments such as catalases. The dead hairs take the colour exactly like normal wool. At the same time 35 the strength and elasticity are increased.

If cotton or other fibers produced from a vegetable material, such as for instance artificial silk, are treated in a like manner, valuable properties are imparted to them 40 and, quite especially, their power of absorbing colouring matter is greatly increased.

The process according to my invention is 45 applicable to fells, feathers, hairs, cotton, jute, hemp, linen, wool, artificial silk and the like and may be applied at any time such as for instance before spinning before, during or after dyeing, during the finishing and so on.

In practising my invention I prefer proceeding 50 in such a manner that I treat the fibers, feathers or hairs to be rendered active either singly, for instance by burling, or in the lock, in the top or sliver, in the cord or, in the case of fells or textile fabric, in the piece with ferments such as catalases

or reductases and the like. The selection and quantity of the ferments used varies according to the desired result; as a rule very small quantities for instance from 0,1 to 2 per cent will suffice. 60

I have ascertained that a like result cannot be obtained by the aid of such ferments as are exclusively zymotic ferments such as the diastase, or such ferments as are effective in flax-retting or in dyeing with natural indigo in the steeping-trough. 65

I have found it to be of special advantage to further treat the fibers with such materials as favour the vitality (activity) of the ferments employed, such substances 70 being for instance the kinases. If catalase is employed, I prefer adding creatinin as an activating medium.

My novel method is the more important 75 since by the suitable selection of the ferments the fastness of the colours produced on the activated fibers is increased.

Between the known methods of dyeing textile fibers with natural indigo or the like in the steeping trough, which contains certain ferments, and the novel process forming the object of the present invention there is this difference that in the latter process only such ferments are used which do not contain any coloring components. In other 85 words, the ferment is in the nature of an enzyme which will not ferment or decompose starch and albumin.

I claim:

1. The process of increasing the strength, 90 elasticity and absorbent power of textiles, which comprises treating said textiles in a bath containing an oxidase.

2. The process of increasing the strength, 95 elasticity and absorbent power of textiles, which comprises treating said textiles in a bath containing an oxidase and a substance capable of favorably influencing the action of the oxidase.

3. The process of increasing the strength, 100 elasticity and absorbent power of textiles, which comprises treating said textiles in a bath containing a catalase.

4. The process of increasing the strength, 105 elasticity and absorbent power of textiles, which comprises treating said textiles in a bath containing a catalase and a substance capable of favorably influencing the action of the catalase.

5. The process of increasing the strength, 110

elasticity and absorbent power of textiles, which comprises treating said textiles in a bath containing an oxidase and creatinin.

6. The process of increasing the strength, elasticity and absorbent power of textiles, which comprises treating said textiles in a bath containing a catalase and creatinin.

7. The process of increasing the strength, elasticity and absorbent power of artificial 10 silk, which comprises treating said artificial silk in a bath containing an oxidase.

8. The process of increasing the strength, elasticity and absorbent power of artificial 15 silk, which comprises treating said artificial silk in a bath containing an oxidase and a substance capable of favorably influencing the action of the oxidase.

9. The process of increasing the strength, elasticity and absorbent power of artificial

silk, which comprises treating said artificial 20 silk in a bath containing catalases and a substance capable of favorably influencing the action of the catalases.

10. The method of treating artificial silk which comprises treating said fiber with cat- 25 alases.

11. The method of treating artificial silk which comprises treating said fiber with cat- 30 alases in the presence of creatinin.

12. As an article of manufacture, artificial 35 silk which has been treated with catalases.

13. As an article of manufacture, artificial silk which has been treated with catalases in the presence of creatinin.

In testimony whereof I have hereunto 35 set my hand.

DR. JOHANNES KORSELT.